# EUROPEAN PATENT SPECIFICATION

(11) **EP 0 635 080 B1**
(45) Date of publication and mention of the grant of the patent: **12.03.1997**
(21) Application number: 93907878.8
(22) Date of filing: 01.04.1993
(51) Int. Cl.: D21C 3/20

(54) **METHOD OF PRODUCING PULP**
VERFAHREN ZUR ZELLSTOFFHERSTELLUNG
PROCEDE DE PRODUCTION DE PATE

(30) Priority: 06.04.1992 US 863977; 17.02.1993 US 19113
(43) Date of publication of application: 25.01.1995
(73) Proprietor: A. AHLSTROM CORPORATION, 29600 Noormarkku (FI)
(72) Inventor: EBELING, Kari, SF-02100 Espoo (FI); HENRICSON, Kaj, SF-00330 HELSINKI (FI); LAXEN, Torolf, SF-00830 Helsingfors (FI); LÖNNBERG, Bruno, SF-20500 Abo (FI)
(74) Representative: Füchsle, Klaus, Dipl.-Ing.
(86) International application number: FI9300137
(87) International publication number: WO9320279

(56) References cited:
- WO-A-82/00483
- DE-A- 2 644 155
- US-A- 3 585 104

## Description

The present invention relates to a new method of producing chemical pulp. The invention is an improvement in solvent cooking methods (e.g. organic solvent digestion), often referred to as "solvent pulping", being generally as described in U.S.-A- 3,585,104.

Wood comprises cellulosic fibres with lignin both inside the fibres and between the fibres, bonding the fibres together. In order to carefully separate the fibres from each other, the lignin must be removed from between the fibres, the removal usually being accomplished by dissolving the lignin. Generally the cooking liquors consist of sodium hydroxide (i.e. soda cook), sodium hydroxide containing sodium sulphide (i.e. sulphate or kraft cook, also called alkaline cook), or, for example, sulphite ions sulphite cook, also called acid sulphite cook). Lignin can also be removed by some organic solvents (hence the commercial name organosolv-process), the best known of which are methanol and ethanol. Formic acid is another proposed organic solvent.

Methanol and ethanol can be utilized as solvents in both alkaline and acid cooks. The advantage of acid cooks is the simple recovery of the chemicals, as wood contains acids that make the cook acid, when only methanol or ethanol are used as solvents. The disadvantage of acid cooks is the poor quality of the produced pulp, because the cellulosic fibres will, to some extent, degrade in acid treatment. In alkaline cooks the quality of the produced pulp will remain good, but the problem in alkaline cooks is the recovery of chemicals. Some alkali, mostly a sodium-based alkali, will firstly have to be added into the cook and then recovered and used again. A known alkaline organic solvent process is the "Organo-cell-process", presently being used in Germany, in which process the cook is a soda-methanol cook.

According to the present invention, it has been determined that during solvent pulping acids are formed in the very beginning of the cook. The pH of the cook can be kept in the desirable range (generally neutral) by removing the acids from the beginning of the cook, i.e. almost immediately after they are formed. By keeping the pH generally neutral, the pulp quality is enhanced, both for continuous and batch cooking processes. This is accomplished, in general, by countercurrent flow during continuous cooking, and in batch cooking by withdrawing solvent from the batch digester after a predetermined time from the start of the cook (and perhaps periodically thereafter), while the cook continues after the solvent withdrawal, with new solvent added.

According to one aspect of the present invention there is provided a method of producing cellulose pulp from comminuted cellulosic fibrous material by organic solvent pulping comprising the step of (a) controlling the pH of the material during cooking so that it is generally neutral by removing acids formed at the start of the cook together with organic solvent used in the cook and by adding alkali to the cellulosic fibrous material in an amount sufficient to maintain the pH at the desired value. This method may be practised utilizing a treatment vessel, comprising further the further steps of: (b) Causing the cellulosic fibrous material to flow in a first direction into the treatment vessel, and to be removed from the treatment vessel in the same, first, direction, whereby the needed amount of alkali is added to the material prior to the treatment vessel; and (c) introducing an organic solvent containing liquid stream to dissolve the lignin of the cellulosic fibrous material into the treatment vessel in a second direction, opposite the first direction. Step (a) is practised by removing the acids formed during pulping, together with spent organic solvent, from the treatment vessel.

A method of producing cellulose pulp from comminuted cellulosic material by organic solvent pulping is known from DE-B-2644155. Further, such a method is also known from WO-A-8200483.

It is the primary object of the present invention to provide effective solvent pulping with a stable pH.

This object is solved in accordance with the present invention by a method including the features of claim 1. Detailed embodiments of this method are defined in the dependent claims.

According to another aspect of the present invention, there is provided a method of producing cellulosic pulp from comminuted cellulosic fibrous material by solvent pulping comprising the steps of:
causing the comminuted cellulosic fibrous material to flow in a first stream in a first direction;
causing a stream of organic solvent to flow into operative contact with the comminuted cellulosic fibrous material countercurrent to the first stream, that is in a second direction, opposite the first direction throughout the area of operative contact between them, which causes organic acids to be produced as the organic solvent dissolves the lignin from the cellulosic fibrous material; and
removing organic acids formed during solvent pulping from intimate contact with the cellulosic fibrous material along with the countercurrent flow of organic solvent.

This and other aspects of the invention will become clear from an inspection of the detailed description of the invention, and from the appended claims.

The method of producing pulp according to the invention will become clear from the detailed description, with reference made to the accompanying drawings, of which:
Figure 1 is a schematic of an exemplary embodiment of a cook/extraction process according to the invention;
Figure 2 is a schematic of another exemplary embodiment of a cook/extraction process according to the invention;
Figure 3 is a schematic of an exemplary embodiment of the washing stage subsequent to the cook/extraction process;
Figure 4 is a schematic of an exemplary embodiment of solvent recovery process according to the invention;
Figure 5 is a schematic of another exemplary embodiment of a cook/extraction process according to the invention;
Figure 6 and 7 illustrate the change of pH as observed when examining the cook/extraction process of Figure 1;
Figure 8 is a schematic diagram illustrating apparatus for practising a method according to the present invention;
Figure 9 is a schematic of an exemplary embodiment of solvent and alkali recovery process according to the invention; and
Figure 10 is a possible process alternative of an application of the invention; and
Figure 11 is a possible process alternative of an application of the invention on an industrial scale.

Figure 1 illustrates a schematic representation of the principle of a countercurrent cook/extraction treatment vessel/stage 20 according to the invention. The number 10 refers to comminuted cellulosic fibrous material (e.g. wood) being fed into the process and the number 11 refers to cellulosic fibres of the wood, produced by dissolving and extracting lignin from the wood. The number 12 refers to the organic solvent being fed to the process and the number 13 refers to the spent organic solvent being exhausted from the process, with dissolved lignin also present. The process of Fig. 1 was examined in laboratory conditions with the surprising result shown in Fig. 6.

In a normal organosolv cook of softwood the pH followed the curve 100. As the acids in the wood are dissolved the pH decreases in about 15 minutes to 3.6 - 3.5 and remains at this level for the rest of the cook. In an organosolv cook of hardwood, the pH decreases to 3.8 - 4.0. This means that all acids either form or dissolve in the initial phase of the cook. The poor fibre strength produced is due to the acid conditions in the cook. The low pH in the cook of softwood may also result in condensation of lignin which prevents dissolution of lignin.

In a countercurrent organosolv cook according to the present invention the pH followed the curve 101. In the initial stage of the extraction the pH was noticed to decrease sharply, but then to quickly increase to almost the original level of about 5.5. The reason for this must be that the organic acids present in the wood are initially dissolved into the solvent, and as the process is a countercurrent one, the acids are washed away with the solvent during the later stages of the cook. The pH can be maintained on an almost neutral level during the cook without using alkali. The quality of the pulp is improved because of reduced acidity during the later stages of the cook.

In 1989, at the Solvent Pulping Conference, Quinde gave a lecture on what happens to the extractives of pine in a methanol cook (80% methanol, 205 °C). He concluded, that 90% of resin acids and about one fourth of fatty acids are dissolved during the first five minutes. This supports the surprising result that the fall of the pH can be prevented by a countercurrent flow of cooking liquor, as shown in Fig. 6 (or by removing the formed acids shortly after production in a batch digester). Obviously the remaining resin and fatty acids are removed due to the countercurrent nature of the process. Thus, according to the invention, the pH of the extraction process can be controlled by removing the organic acids, formed during the process, together with the always countercurrent flow of solvent.

The results from the experiments described in Fig. 6 can be further explained by means of Fig. 7.

On region C of Fig. 7 the pH is below 4.5 whereby the quality of the pulp deteriorates. In the case of a normal ethanol cook most of the time the pH is below this level and this results in poor quality of pulp. This case is represented by curve 104 in Fig. 7. However, when utilizing a countercurrent cooking procedure as according to the invention, the pH remains below the minimum desirable level (line 105) for pH during the cook only a short period of time. Since the time during which the pH is too low is short, a pulp of good quality is produced. This is represented by curve 103 in Fig. 7.

The pulp quality can be further improved by adding alkali to the countercurrent cook at the beginning of the cook. This case is shown in Fig. 7 by curve 102. The alkali added in the beginning increases the pH and acids formed or dissolved neutralize the cook and the pH decreases to an almost neutral value during the countercurrent cook. There is a maximum desirable pH, represented by line 106, which is desirably not exceeded (region A in Fig. 7) because then the amount of alkali that has to be recovered becomes so high that the recovery system becomes expensive. By controlling the pH in this way within region B, a pulp of good quality is produced.

It can be said that it is most advantageous to keep the pH of the solvent cooking process in the range of 4.5 - 12, but it can be momentarily allowed to decrease below 4.5 or increase above 12 at the beginning of the cook. The minimum is reached when no alkali is used and the maximum when alkali is used. Alkali can also be added in such an amount as to maintain the pH of the cook between the minimum and maximum limits.

A countercurrent extraction according to Fig. 2 ensures that the pH does not decrease at the initial stages of the cook/extraction 20. An addition of alkali 14, for example CaO, Na₃CO₃ or NaOH, or a combination thereof, to the wood material 10 being fed into the cook, neutralizes the initial stage of the cook and so prevents the pH from falling. Thus the pH is prevented from decreasing to the level of about 3-4, where hydrolysis would degrade the cellulosic fibres. The amount of acid forming at the initial stages of the cook is 8-20 kg/ton of pulp, and an amount of alkali corresponding to the amount of acid is added, if the pH is to be kept out of the acid range (e.g. generally neutral, for example a pH of about 6.5 - 7.5). Due to the essentially completely countercurrent nature of the cook there is some alkali present at the initial stages of the cook 20, but it is then washed away and removed with the dissolved lignin in stream 13.

When effecting countercurrent cooks in laboratory conditions it was also discovered that a high ethanol or methanol content (e.g. 70% or more) in the organic solvent containing liquid gives a better delignification result. It has usually been presumed, that due to the water included in the wood, the ethanol content could be 50% at the most. When a countercurrent cook is effected, the ethanol content can be substantially increased to exceed 50% of the organic solvent containing liquid by maintaining a high ethanol content in the inlet streams 12 (Figs. 1 and 2). According to the invention, the water is washed away at the beginning of the cook and is removed with streams 13. Thus the countercurrent cook gives a possibility of both controlling the pH and increasing the content of the organic solvent.

The residual solvent in the stream of fibres subsequent to the extraction 20 must be washed away as shown in Fig. 3. The stream 11 of fibres is a mixture of organic solvents and wood fibres. Because of the countercurrent nature of the cook/extraction, it can be presumed that the fibres are suspended in nearly pure solvent. In the washing stage 21 the solvent is washed away with washing liquid 16, mostly water. The result is a wood fibre-water suspension 15 and a solution 17 of water and solvent, mostly a mixture of water and ethanol or methanol.

The solvent is recovered from stream 17 by a process according to, for example, Fig. 4. The solution 17 of water and solvent is directed to distillation apparatus 22, where the water 18 and solvent 12 are separated. The solvent 12 is directed to cook 20. As is shown in Fig. 4, it is possible to effect a wash in 21 with water and still maintain a high ethanol and/or methanol content in the actual cook 20. The pulp, if any, still in the form of chips prior to the wash, is fiberized prior to the wash to optimize the wash. The organic solvent 12 preferably has a substantially greater than 30% methanol and/or ethanol content.

Fig. 5 illustrates a process more developed than heretofore described. The wood 30 introduced into the process is heated at the beginning of the cook by feeding steam 31 in the wood material in presteamer 23. Alkali 32 is at the same time introduced into the wood material to increase the pH at the initial stage of the cook. A catalyst 33 can be introduced during either the pretreatment 23 or at the beginning of the cook 20 to enhance the dissolving of lignin. A commonly used catalyst in acid process is CaCl₂. The Ca²⁺ ions are advantageous to the process, but on the other hand the amount of acid is detrimentally increased in the reaction 2Cl- + 2H+ → 2HCl. Organic bases, such as amine, can be used as catalysts in acid, neutral and alkaline processes. Ethanol or methanol 34 is added to make up for the losses of solvent in the process.

The process has further been complemented by treatment of the lignin-containing outlet liquid 36. Naturally, the outlet liquids 13 of the previous embodiments can also be treated accordingly. The outlet stream 36 of solvent from the cook 20 mostly contains solvent, polysaccharides, lignin and water. The mixture 36 is directed to distillation/evaporation stage 24, where the solvent, mostly ethanol and/or methanol 37, is separated from the water 38 and lignin and polysaccharide material 39. The solvent 37 can be returned to the cook 20 together with the solvent 12 from the distillation stage 22, while the water and lignin material are directed to combustion apparatus 25 or other treatment device. One possibility is to separate the lignin and to produce, for example, vanillin from the separated lignin. The added alkali 32, if any, is directed to combustion apparatus 25 and can thereafter be reused, or, if desired, removed. Removal is typically practised if the amount of the added alkali is small, e.g. 10-50 kg/ton of pulp.

In a laboratory test producing pulp of good quality, CaCl₂ was utilized as catalyst, the amount of which was 5-50 g/l (that is about 5-50 grams of catalyst per litre of material being treated). The temperature of the cook was 195 °C and the duration of the cook 20 was 3 hours. Other possible catalysts, besides Ca++, are Mg++ and Na+. For the lignin extraction it is advantageous that the wood is impregnated with alkali (14, 32), as this causes the wood to swell and thereby improves the extraction of lignin.

Ethanol is probably a better solvent than methanol for the practice of the invention, but the deacetylation that occurs in the wood produces some methanol. Thus there is always some methanol present in the process, even if the only fresh solvent 34 is ethanol.

The invention can be applied to numerous cooks, both batch cooks and continuous cooks. The invention can, for example, be utilized in continuous digesters with a pretreatment zone or in continuous digesters with a separate pretreatment vessel. When the invention is practised with batch digesters, the acids produced at the beginning of the cook can be removed by withdrawing solvent from the digester after a predetermined time (e.g. about 5 - 10 minutes, but dependent upon material being cooked, the exact composition of the organic solvent, etc.) - the produced acids being removed with the solvent - and introducing at least some new solvent. While normally not necessary since most of the acids are produced within the first five minutes or so, the withdrawal and replacement procedure can be practised periodically if desirable. The pH during batch cooking can alternatively, or in addition, be maintained generally neutral during the initial stages of the cook by adding alkali to the material prior to or simultaneously with introduction into the digester.

The invention may be further illustrated by the following examples.

### Example

A series of laboratory tests on softwood were performed to study the method. In laboratory the organosolv cooking process was performed as follows:

### Step 1:

The chips were pretreated in a pretreatment liquor consisting of NaOH dissolved in water. The pretreatment time was about 30 minutes and the temperature 120 °C. The idea of the pretreatment step was to cause the fibre to swell so as to enhance the subsequent ethanol extraction step. Another reason for the pretreatment step was to enable the addition of alkali to the chips to keep the pH at a sufficiently high level during the rest of the cook.

During the pretreatment step the amount of alkali was varied between 0.25 to 1.50 mol NaOH/l. It was found that when the amount of alkali was below 0.25 mol NaOH/l the delignification was insufficient and the amount of unfiberized wood high. At alkali levels above 1.00 mol NaOH/l the yield loss in the cook became too high. Probably the amount of alkali actually needed depends on type of wood used. For the tested Scandinavian spruce the optimal alkali level was between 0.5 and 1.0 mol NaOH/l.

### Step 2:

The chips were removed from the pretreatment liquor by lifting the chips out. It was found that about 30 - 70 kg of NaOH per ton of pulp was entrained with the chips.

Alkali had also been consumed in the pretreatment vessel. The consumption was 50 - 300 kg NaOH per ton of pulp.

### Step 3:

Subsequent to steps 1 and 2 the chips were taken to a countercurrent ethanol extraction step. The duration of this solvent extraction step was about 120 minutes and the temperature 185 °C. Anthraquinone was added to the solvent to improve delignification. The added amount of anthraquinone was between 0 and 1.0 mmol.

The strength of the ethanol solvent was varied between 25% and 100%. The lowest residual lignin contents were achieved when the ethanol content was between 40 and 70% in the liquid phase. When being tested for bleachability and pulp properties, the pulp was found to have pulp properties close to those of kraft pulp regarding both bleachability and strength.

Figure 8 shows an apparatus with which the process of example 1 can be performed. The apparatus comprises a conventional chips bin 201 connected by a conventional low pressure feeder 202 to a conventional horizontal steaming vessel 203, which in turn is connected by a conventional chute to a conventional high pressure feeder 204. Wood chips are first steamed and preheated and then taken through the first pressure feeder 204 in line 205 to the pretreatment vessel 206 in which the chips are treated in an alkaline solution. The alkaline solution is introduced into the system in line 207. A conventional liquid/ material separator system is provided at the top of the vessel, with withdrawn liquid recirculated via line 208 to the inlet high pressure port of the feeder 204. The alkali can come from one or several of the following sources:
- waste water from alkaline bleaching stages, for example, E or P stages;
- NaOH, either brought fresh to the mill or manufactured at the mill by causticizing Na₂CO₃; and/or
- Na₂CO₃ if the alkalinity needed is so low that only part of the alkali must be NaOH.

From the pretreatment vessel 206 the chips are taken to the extraction zone 215 in the second pressure vessel 213 in which the pressure is much higher than in pressure vessel 206. The chips material passes via line 211 to the top of the vessel 213 from a high pressure feeder 209 in the bottom of the pretreatment vessel 206. A conventional liquid/material separator system is provided at the top of the vessel 213, with withdrawn liquid recirculated via line 212 to the inlet high pressure port of the feeder 209. In order to control the temperature of the recirculating liquid so as to minimize the possible adverse effects on the high pressure feeder 209, the liquid is passed through a heat exchanger 210.

The second vessel 213 preferably consists of two zones: (1) zone 215 in which the chips are extracted with ethanol/methanol; and (2) zone 216 in which the chips are washed before being discharged from the vessel.

Filtrate from a subsequent washing or bleaching step is used as washing liquid. The washing liquid is introduced into the bottom of the vessel 213 through line 218. The pulp at the bottom of the vessel 213 is washed and discharged into line 219.

The ethanol and/or methanol is added at a point above the washing zone 216 in line 217. The ethanol is introduced at such a strength and amount that optimal extraction conditions are achieved in the extraction zone 215. If necessary, water can be separated from the circulation 220 by distillation to control methanol/ethanol strength in the extraction zone 215.

The extraction liquor is withdrawn from the extractor/digester 213 into a withdrawal conduit 214. The withdrawn liquor containing the alkali used, the ethanol/methanol used and the dissolved lignin, is taken to recovery.

A simplified recovery system for solvent and alkali is shown in Fig. 9. The extraction liquor 214 from Fig. 8 is treated in the following steps: (a) Ethanol/methanol separation (250). The solvent is then reused in the extraction vessel 213. (b) Evaporation (252) in which water is separated. (c) Combustion (254) of lignin and polysaccharides.

During combustion, a melt (255) consisting essentially of Na₂CO₃ is produced. This melt is dissolved in water and used as a Na₂CO₃ containing liquid in the pretreatment vessel 206 or causticized to NaOH before using in the pretreatment vessel 206. If the Na₂CO₃ amount is small it does not have to be reused.

If the produced pulp is to be chlorine free, the pulp can be bleached with oxygen, ozone and peroxide. Fig. 10 illustrates a diagram of a process in which the initial bleaching is effected by oxygen and the actual final bleaching by ozone and peroxide.

In the system of Fig. 10, the wood chips 300 that are introduced into the process are first heated by feeding steam 301 to the wood material to a pretreatment vessel 323. Alkali 302 is at the same time introduced into the wood material so that the chips are treated at a pH of 11 - 12. The alkali is obtained from the bleach plant effluents, which contain 40 - 120 kg of NaOH/adt. If the volume of the effluent is too big, the effluent has to be evaporated in order to reduce the volume. Additional alkali is brought if needed in the form of NaOH or Na₂CO₃.

After pretreatment 323 the chips 310 are introduced to the extraction stage 320 where some methanol and/or ethanol 312' may be added in the beginning to control the liquor- to - wood ratio, or to increase the content of methanol/ethanol in the beginning of the extraction process 320.

After extraction the chips 311 are washed with the bleach plant effluents 302', 303, 304, which may be acid or alkali depending on how the bleaching has done. If possible, the acid filtrates 303 and 304 are used in the washing 321 and the alkali filtrate 302 in chips pretreatment 323. The washing liquid 317 containing solvent may have to be strengthened by distillation 322 before adding methanol and/or ethanol 312 to the extraction stage 320.

The pulp 315 from the washing stage is introduced into the bleach plant 330 in which the pulp is bleached in the sequence OZP.

After the extraction stage 320 the waste liquor 306 is recovered, evaporated and combusted. If the alkali amount is low, the Na₂CO₃ formed in the recovery process is removed from the mill and fresh NaOH is brought in. Some of the Na₂CO₃ may be used in the pretreatment stage. If the amount of alkali in the effluent stream is large it is probably more practical to causticize the formed Na₂CO₃ to NaOH and thus generate new NaOH for bleaching and pretreatment at the mill.

### Example

In one successful test, the wood was pretreated with a mixture of 75 % Na₂CO₃ and 25 % NaOH in amount that corresponds about 200 kg Na/adt expressed as NaOH. This means that about 50 kg/adt of NaOH was used and the rest was Na₂CO₃.

The amount of NaOH needed in the bleaching sequence OZEP is also about 50 kg/adt. Thus all alkali needed in the pretreatment of the chips in the form of NaOH is received from the bleach plant effluent water. The rest of the alkali can be used as Na₂CO₃ which is the form of the Na when burning the residual liquor in a recovery boiler.

Thus, a mill does not need any causticizing plant, but uses Na₂CO₃ from the combustion of spent liquor and NaOH from bleach plant effluents.

Filtrates from the bleach plant can be used to dissolve the Na₂CO₃ from the recovery boiler thus further reducing the water effluent volume.

Fig. 11 also illustrates a schematic technical diagram of a process in which the initial bleaching is effected by oxygen and the actual final bleaching by ozone and peroxide.

While the invention has been described in connection with what is presently considered to be the most practical and preferred embodiment, it is to be understood that the invention is not to be limited to the disclosed embodiment, but on the contrary, is intended to cover various modifications and equivalent arrangements included within the scope of the appended claims.

## Claims

1. A method of producing cellulose pulp from comminuted cellulosic fibrous material by organic solvent pulping, wherein
(a) the comminuted cellulosic fibrous material is pretreated with alkaline aqueous solution to swell the fibrous material in order to improve solvent penetration and to increase the pH so that the pH of the material during solvent pulping is maintained at least neutral;
(b) the pretreated cellulosic fibrous material is treated with an organic solvent-containing liquid, and the lignin of the material is extracted with the solvent; and that
(c) the treated cellulosic fibrous material is washed to remove and extract the dissolved lignin and to effect removal of undesired chemicals thereform.

2. A method according to claim 1, wherein steps (b) and (c) are performed by countercurrent extraction and countercurrent washing.

3. A method according to claim 1, wherein steps (a), (b) and (c) are practised substantially continuously.

4. A method according to claims 2 or 3, wherein steps (b) and (c) are practised utilizing a treatment vessel, whereby
- the cellulosic fibrous material is caused to flow in a first direction into the treatment vessel, and to be removed from the treatment vessel in the same, first, direction, whereby the needed amount of alkali is added to the material prior to the treatment vessel; and
- a stream of liquid containing organic solvent is introduced into the treatment vessel in a second direction, opposite to the first direction, to dissolve the lignin of the cellulosic fibrous material; and the acids formed during pulping are removed with the countercurrent flow of spent organic solvent from the treatment vessel.

5. A method according to claim 1, wherein the spent organic solvent is extracted from step (b) and treated to remove organic solvent from the dissolved material therein.

6. A method according to claim 5, wherein the separated organic solvent from the separation step is introduced to be used as organic solvent in step (b).

7. A method according to claim 5, wherein the separated material removed from the organic solvent in the separation step is combusted to produce a melt containing Na₂CO₃ and the melt is dissolved in water to produce a liquid, which is used as alkali without or after causticization and added to the cellulosic fibrous material in step (a).

8. A method according to claim 1, wherein some of the chemicals removed during washing comprise organic solvent, which is separated from the washing liquid and introduced into step (b).

9. A method according to claim 8, wherein the organic solvent is separated from the washing liquid by distillation.

10. A method according to claim 1, wherein the cellulosic fibrous material is steamed prior to or during step (a).

11. A method according to claim 1, wherein a catalyst to enhance dissolving of lignin is introduced into the cellulosic fibrous material prior to step (b).

12. A method according to claim 11, wherein the catalyst is selected from the group consisting essentially of salts of alkali-earth metals, anthraquinone and organic bases, and in that about 5-50 grams of catalyst is added per litre of material being treated.

13. A method according to claim 1, wherein the pulping is practised in a batch digester by removing spent solvent containing formed acids, from the digester shortly after formation of the vast majority of acids at the start of the cook.

14. A method according to claim 1, wherein the organic solvent in the organic solvent-containing liquid is selected from the group consisting essentially of methanol, ethanol, and mixtures of methanol and ethanol.

15. A method according to claim 14, wherein the amount of methanol, ethanol, and mixtures of methanol and ethanol, is substantially greater than 50 % of the total amount of the solvent-containing liquid.

16. A method according to claim 1, wherein NaOH is used as alkali in step (a).

17. A method according to claim 16, wherein also Na₂CO₃ is used as alkali in step (a).

18. A method according to claim 1, wherein the cellulosic fibrous material in step (c) is washed with water.

## Patentansprüche

1. Verfahren zur Herstellung von Zellstoff aus zerkleinertem zellulosehaltigem Fasermaterial durch Aufschluß mit organischem Lösemittel, **dadurch gekennzeichnet, daß**
(a) das zerkleinerte zelluloschaltige Fasermaterial mit alkalischer wäßriger Lösung zur Schwellung des Fasermaterials vorbehandelt wird, um das Eindringen von Lösemittel zu verbessern und den pH anzuheben, so daß der pH des Materials während des Solvent-Aufschlusses zumindest neutral bleibt;
(b) das vorbehandelte zelluloschaltige Fasermaterial mit einer organisches Lösemittel enthaltenden Flüssigkeit behandelt wird und das Lignin des Materials mit dem Lösemittel extrahiert wird; und daß
(c) das behandelte zelluloschaltige Fasermaterial gewaschen wird, um das aufgelöste Lignin zu entfernen und extrahieren und um die Beseitigung unerwünschter Chemikalien daraus zu bewerkstelligen.

2. Verfahren nach Anspruch 1, **dadurch gekennzeichnet, daß** die Schritte (b) und (c) durch Gegenstrom-Extraktion und -Wäsche ausgeführt werden.

3. Verfahren nach Anspruch 1, **dadurch gekennzeichnet, daß** die Schritte (a), (b) und (c) im wesentlichen kontinuierlich praktiziert werden.

4. Verfahren nach Anspruch 2 oder 3, **dadurch gekennzeichnet, daß** die Schritte (b) und (c) durch Anwendung eines Behandlungsbehälters praktiziert werden, wobei
- das zelluloschaltige Fasermaterial veranlaßt wird, in einer ersten Richtung in den Behandlungsbehälter zu fließen und aus dem Behandlungsbehälter in der gleichen ersten Richtung entfernt zu werden, wobei die gebrauchte Alkalimenge dem Maleriai vor dem Behandlungsbehälter zugesetzt wird; und
- ein organisches Lösemittel enthaltender Flüssigkeitsstrom in den Behandlungsbehälter in einer zweiten, der ersten Richtung entgegengesetzten Richtung eingeführt wird, um das Lignin des zellulosehaltigen Fasermaterials aufzulösen; und die beim Aufschluß gebildeten Säuren mit dem Gegenstrom verbrauchten organischen Lösemittels aus dem Behandlungsbehälter entfernt werden.

5. Verfahren nach Anspruch 1, **dadurch gekennzeichnet, daß** das verbrauchte organische Lösemittel von Schritt (b) extrahiert und behandelt wird, um organisches Lösemittel aus dem aufgelösten Material darin zu entfernen.

6. Verfahren nach Anspruch 5, **dadurch gekennzeichnet, daß** das abgeschiedene organische Lösemittel von der Abscheidestufe eingeführt wird, um als organisches Lösemittel in Schritt (b) benutzt zu werden.

7. Verfahren nach Anspruch 5, **dadurch gekennzeichnet, daß** das abgeschiedene, in der Abscheidestufe vom organischen Lösemittel entfernte Material verbrannt wird, um eine Na₂CO₃ haltige Schmelze zu erzeugen, und die Schmelze in Wasser aufgelöst wird, um eine Flüssigkeit zu produzieren, die als Alkali ohne oder nach Kaustizierung verwendet und dem zellulosehaltigen Fasermaterial in Schritt (a) zugeführt wird.

8. Verfahren nach Anspruch 1, **dadurch gekennzeichnet, daß** einige der während der Wäsche entfernten Chemikalien organisches Lösemittel enthalten, das aus der Waschflüssigkeit abgeschieden und Schritt (b) zugeführt wird.

9. Verfahren nach Anspruch 8, **dadurch gekennzeichnet, daß** das organische Lösemittel durch Destillation aus der Waschflüssigkeit abgeschieden wird.

10. Verfahren nach Anspruch 1, **dadurch gekennzeichnet, daß** das zelluloschaltige Fasermaterial vor oder während Schritt (a) gedämpft wird.

11. Verfahren nach Anspruch 1, **dadurch gekennzeichnet, daß** ein Katalysator zur Verbesserung der Auflösung von Lignin dem zellulosehaltigen Fasermaterial vor Schritt (b) zugeführt wird.

12. Verfahren nach Anspruch 11, **dadurch gekennzeichnet, daß** der Katalysator aus einer Gruppe gewählt wird, die im wesentlichen aus Salzen von Alkali-Erdmetallen, Anthrachinonen und organischen Basen besteht, und daß ungefähr 5 - 50 Gramm Katalysator pro Liter Behandlungsgutes zugesetzt werden.

13. Verfahren nach Anspruch 1, **dadurch gekennzeichnet, daß** der Aufschluß in einem diskontinuierlichen Kocher praktiziert wird, indem verbrauchtes Lösungsmittel enthaltende gebildete Säuren aus dem Kocher entfernt werden, sobald sich die überwiegende Mehrheit der Säuren zu Beginn des Aufschiusses gebildet hat

14. Verfahren nach Anspruch 1, **dadurch gekennzeichnet, daß** das organische Lösemittel in der organisches Lösemittel enthaltenden Flüssigkeit aus einer Gruppe gewählt wird, die im wesentlichen aus Methanol, Äthanol, und Mischungen von Methanol und Äthanol besteht.

15. Verfahren nach Anspruch 14, **dadurch gekennzeichnet, daß** die Menge an Methanol, Äthanol und Mischungen von Methanol und Äthanol wesentlich grösser als 50 % der Gesamtmenge der Lösemittel enthaltenden Flüssigkeit ist.

16. Verfahren nach Anspruch 1, **dadurch gekennzeichnet, daß** NaOH als Alkali in Schritt (a) verwendet wird.

17. Verfahren nach Anspruch 16, **dadurch gekennzeichnet, daß** auch Na₂CO₃ als Alkali in Schritt (a) verwendet wird.

18. Verfahren nach Anspruch 1, **dadurch gekennzeichnet, daß** das zelluloschaltige Fasermaterial in Schritt (c) mit Wasser gewaschen wird.

## Revendications

1. Procédé de production de pâte de cellulose à partir de matière fibreuse cellulosique désintégrée par réduction en pâte au solvant organique, dans lequel
(a) la matière fibreuse cellulosique désintégrée subit un prétraitement avec une solution aqueuse alcaline de façon à faire gonfler la matière fibreuse afin d'améliorer la pénétration du solvant et à augmenter le pH pour que le pH de la matière, au cours de la réduction en pâte du solvant, soit maintenu au moins neutre;
(b) la matière fibreuse cellulosique prétraitée est traitée avec un liquide contenant un solvant organique, et la lignine de la matière est extraite avec le solvant; et
(c) la matière fibreuse cellulosique traitée est lavée pour enlever et extraire la lignine dissoute et afin d'en effectuer l'élimination des produits chimiques indésirables.

2. Procédé selon la revendication 1, dans lequel les étapes (b) et (c) sont accomplies par extraction à contre-courant et lavage à contre-courant.

3. Procédé selon la revendication 1, dans lequel les étapes (a), (b) et (c) sont accomplies sensiblement de manière continue.

4. Procédé selon les revendications 2 ou 3, dans lequel les étapes (b) et (c) sont accomplies en utilisant une enceinte de traitement afin que :
- la matière fibreuse cellulosique soit amenée à s'écouler dans une première direction dans l'enceinte de traitement, et soit enlevée de l'enceinte de traitement dans la même, première, direction, de façon que la quantité exigée d'alcali soit ajoutée à la matière avant l'enceinte de traitement; et
- un courant de liquide contenant un solvant organique est introduit dans l'enceinte de traitement dans une seconde direction, opposée à la première, afin de dissoudre la lignine de la matière fibreuse cellulosique; et les acides formés au cours de la réduction en pâte sont éliminés avec l'écoulement à contre-courant du solvant organique utilisé à partir de l'enceinte de traitement.

5. Procédé selon la revendication 1, dans lequel le solvant organique utilisé est extrait de l'étape (b) et traité de façon à enlever du solvant organique de la matière y dissoute.

6. Procédé selon la revendication 5, dans lequel le solvant organique séparé provenant de l'étape de séparation est introduit afin d'être utilisé en tant que solvant organique au cours de l'étape (b).

7. Procédé selon la revendication 5, dans lequel le matériau séparé enlevé du solvant organique au cours de l'étape de séparation est brûlé afin de produire un bain fondu contenant du Na₂CO₃ et ce bain fondu est dissout dans l'eau afin de produire un liquide, qui est utilisé en tant qu'alcali sans ou après caustification et qui est ajouté à la matière fibreuse cellulosique dans l'étape (a).

8. Procédé selon la revendication 1, dans lequel quelques-uns des produits chimiques enlevés lors du lavage comprennent un solvant organique, qui est séparé du liquide de lavage et introduit dans l'étape (b).

9. Procédé selon la revendication 8, dans lequel le solvant organique est séparé, par distillation, du liquide de lavage.

10. Procédé selon la revendication 1, dans lequel la matière fibreuse cellulosique est traitée à la vapeur avant ou au cours de l'étape (a).

11. Procédé selon la revendication 1, dans lequel un catalyseur, pour améliorer la dissolution de la lignine, est introduit dans la matière fibreuse cellulosique avant l'étape (b).

12. Procédé selon la revendication 11, dans lequel le catalyseur est sélectionné parmi le groupe comprenant essentiellement des sels des métaux alcalino-terreux, l'anthraquinone et des bases organiques, et environ 5 - 50 grammes de catalyseur sont ajoutés par litres de matériau en cours du traitement.

13. Procédé selon la revendication 1, dans lequel la réduction en pâte est effectuée dans un lessiveur discontinu en retirant du lessiveur le solvant utilisé contenant des acides formés, peu de temps après la formation de la grande majorité d'acides au commencement de la cuisson.

14. Procédé selon la revendication 1, dans lequel le solvant organique contenu dans le liquide contenant du solvant organique est choisi parmi le groupe qui comprend essentiellement le méthanol, l'éthanol, et des mélanges de méthanol et d'éthanol.

15. Procédé selon la revendication 14, dans lequel la quantité de méthanol, d'éthanol et des mélanges de méthanol et d'éthanol est sensiblement supérieure à 50% de la quantité totale du liquide contenant du solvant.

16. Procédé selon la revendication 1, dans lequel on utilise NaOH en tant qu'alcali au cours de l'étape (a).

17. Procédé selon la revendication 16, dans lequel on utilise également Na₂CO₃ en tant qu'alcali au cours de l'étape (a).

18. Procédé selon la revendication 1, dans lequel la matière fibreuse cellulosique dans l'étape (c) est lavée à l'eau.
